

# UNITED STATES PATENT OFFICE.

JOSEPH EUGÉNE PAQUET, OF MONTREAL, QUEBEC, CANADA.

## PROCESS FOR WATERPROOFING FABRICS.

1,306,274.

Specification of Letters Patent. Patented June 10, 1919.

No Drawing.

Application filed September 11, 1918. Serial No. 253,664.

To all whom it may concern:

Be it known that I, JOSEPH EUGÉNE PAQUET, a subject of the King of Great Britain, residing at Montreal, Province of Quebec,

5 Canada, have invented certain new and useful Improvements in Processes for Waterproofing Fabrics; and I do hereby declare that the following is a full, clear, and exact description of the invention, such as will 10 enable others skilled in the art to which it appertains to make and use the same.

The present invention relates to a leather substitute which may be used in the manufacture of footwear, and more particularly 15 to a process for treating fabrics whereby such leather substitute will be made.

Herebefore it has been the practice in the boot manufacture to utilize for the inner soles and stiffeners a hard pressed cardboard 20 made of leather chips, which is sometimes called "leatherboard." The use of this material, however, is unsatisfactory on account of becoming disintegrated by moisture. The product of the present process is not affected 25 by the moisture and will outlast ordinary leather.

In carrying out the present invention a paste is made by dissolving one pound of gluten into two gallons of hot water, to 30 which is added one half pound of glue or gelatin and one pint of boiled linseed oil. Canvas white duck or similar cotton fabrics may be used as the base, but, of course, it is to be understood that any suitable goods or 35 fabrics may be used. The fabric is then submerged in this liquid as formed or the liquid may be applied to the fabric with a brush, after which it is allowed to dry. After the fabric or basic substance is dry, it 40 is again treated with a paste made substantially in the same way as the first mentioned paste, but the quantity of glue or gelatin and

oil is doubled, that is, the composition for the second treatment comprises one pound of gluten dissolved in two gallons of water, 45 and one pound of glue or gelatin and one quart of linseed oil. After this second coating has been applied and dried the fabric will be impervious to moisture.

Whereas I have mentioned the use of 50 gluten, a good substitute therefor may be a light flour, preferably wheat flour.

The proportions above given produce the best results, but the right is hereby reserved to vary the proportions herein given that 55 come within the scope of the present invention.

Having thus fully described my invention, what I claim as new and desire to secure by Letters Patent is:

1. A process of waterproofing fabric consisting in coating the same with a paste including gluten, linseed oil and glue, drying said fabric and then subjecting the same to a second application of a paste including 65 gluten and the double quantity of glue and linseed oil.

2. A waterproof fabric composed of a woven fabric and a composition incorporated therein and occupying the interstices 70 thereof comprising gluten, gelatin and a vegetable oil.

3. A leather substitute comprising a basic member impregnated first with a composition comprising 1 pound of gluten mixed 75 with 2 gallons of hot water,  $\frac{1}{2}$  pound of glue and 1 pint of boiled linseed oil, and again treated with a paste comprising 1 pound of gluten, mixed with 2 gallons of water, 1 pound of glue and 1 quart of linseed oil substantially as and in the manner specified.

In witness whereof I have hereunto set my hand.

JOSEPH EUGÉNE PAQUET.